# EUROPEAN PATENT SPECIFICATION

(11) **EP 0 209 632 B1**
(45) Date of publication and mention of the grant of the patent: **25.07.1990**
(21) Application number: 86103186.2
(22) Date of filing: 10.03.1986
(51) Int. Cl.: B21B 3/00, C22F 1/18, C22C 27/04

(54) **Method for producing an elongate tungsten article**
Herstellungsverfahren für ein langgestrecktes Produkt aus Wolframhartmetall
Méthode pour la fabrication d'un produit long en métal dur detungstène

(30) Priority: 10.07.1985 US 753843
(43) Date of publication of application: 28.01.1987
(73) Proprietor: GTE Products Corporation, Wilmington, DE 19801 (US)
(72) Inventor: Mullendore, James A., Towanda PA 18848 (US); Spencer, James R., Sayre, PA 18840 (US)
(74) Representative: Grünecker, Kinkeldey, Stockmair & Schwanhäusser Anwaltssozietät

(56) References cited:
- EP-A- 0 073 384
- DE-A- 2 156 444
- DE-B- 1 558 821
- DE-B- 1 957 073
- DE-B- 2 242 760
- DE-B- 2 727 892
- FR-A- 1 330 469
- US-A- 3 859 055
- PATENT ABSTRACTS OF JAPAN, vol. 6, no. 120 (M-140)[998], 3rd July 1982

## Description

The present invention relates to a method of producing an essentially elongate article of tungsten heavy alloy material of the type as indicated in the pre-characterising portion of claim 1.

A method of this type is known from DE-B 1 558 821. This prior art document discloses a method for improving the ductility of articles made of tungsten or of tungsten alloys. According to this disclosure, rod-like sintered tungsten blanks are typically heated repeatedly to temperatures from 800 to 1800_{°}C and forged or rolled in order to obtain tungsten crystallites of elongated size.

In the as-sintered condition, tungsten heavy alloys have isotropic properties, that is, the properties are equal in all directions since these alloys consist of nearly spherical tungsten grains in a matric of the alloying elements as nickel and iron, copper or cobalt. In certain applications, as in kinetic energy penetrators, it is desirable to have anisotropic or directional properties to allow for a minimum of fracturing and crack propagation when the penetrator hits a target.

It is the object of the present invention to produce an essentially elongate article of tungsten heavy alloy material of which the tungsten grains have a length to diameter ratio of at least about 2:1. In particular, it is the object of the present invention to produce a tungsten heavy alloy material article which is useful as a kinetic energy penetrator. Kinetic energy penetrators must have strength to resist cracking since high bending stresses which cause cracking are generated when the penetrator hits a target. The target is usually at high obliquity to the path of the penetrator. When the penetrator strikes the target, the penetrator is deflected from its original path and this in effect bends the penetrator and, when the length to the diameter ratio of the tungsten grains is less than about 2:1, the penetrator fractures in a transverse manner. Said fracturing would reduce the penetrator's ability to perforate the target. With the elongated grain structure, that is, of a length to diameter ratio of at least about 2:1, the penetrator is more able to resist fracturing and, therefore, gives better performance.

The above object is achieved by the method as defined in claim 1 wherein the inventive method distinguishes over DE-B 1 558 821 in that the rolling of a press and sintered body having the desired composition is effected in a tandem rolling mill having a succession of rolls stands, each stand consisting essentially of three rolls positioned at substantially 120° to each other so that the gap between the rolls is at a triangle, each stand being rotated about 180_{°} with respect to the adjacent roll stands, the rolling being effected such that the length to diameter ratio of said elongate tungsten grains is at least 2:1.

The above method steps of the inventive method allow for the tungsten heavy metal alloy to be heavily worked without introducing an excessive number of defects to obtain the critical length to diameter ratio.

Preferred embodiments of the inventive method are indicated in the sub-claims.

### Brief description of the drawings

Figure 1 is a photomicrograph taken at about 200x magnification of essentially spherical grain tungsten heavy alloy material in the as-sintered condition.
Figure 2 is a photomicrograph taken at about 200x magnification of essentially spherical grain tungsten heavy alloy material in a slightly worked condition.
Figure 3 is a schematic diagram showing the crack propagation pattern in material of Figures 1 and 2.
Figure 4 is a photomicrograph taken at about 200x magnification of the article manufactured according to this invention.
Figure 5 is a schematic diagram showing where crack propagation would occur in the article manufactured according to his invention.

### DETAILED DESCRIPTION OF THE INVENTION

For a better understanding of the present invention, together with other and further objects, advantages, and capabilities thereof, reference is made to the following disclosure and appended claims in connection with the above described drawings and description of some embodiments of the invention.

The article produced with the method according to the invention is made of tungsten heavy alloy material. The alloy material is essentially tungsten, nickel, and iron. Copper and cobalt can also be present. Generally the tungsten is present in from about 70% to about 98% by weight. It is preferred that the alloy material contain no greater than about 96% by weight tungsten and that the nickel and iron be present in a weight ratio of greater than about 1.5 to 1 of nickel to iron. It is especially preferred that the alloy material contain from about 90% to about 96% by weight tungsten and that the nickel and iron be present in a weight ratio of about 7 to 3 of nickel to iron.

The article generally has a tungsten grain diameter of about 20 to 80 microns.

The tungsten grains have a length to diameter ratio of at least about 2 to 1, and preferably from about 4 to 1 to about 5 to 1. The advantage of this structure it that it is more resistant to fracturing than the more spherical structure. Figures 1 and 2 are photomicrographs of the prior art material. Figure 1 is a photomicrograph taken at about 200x magnification of essentially spherical grain tungsten heavy alloy material in the as-sintered condition. Figure 2 is a photomicrograph taken at about 200x magnification of essentially spherical grain tungsten heavy alloy material in a slightly worked condition, that is, worked to about a 30% reduction in diameter, or a length to diameter ratio of about 1.5 to 1. Figure 2 shows that even with a slight amount of working, there are defects present. Figure 3 is a schematic diagram showing how crack propagation occurs in spherical grain tungsten heavy alloy material. It can be seen from Figure 3 that the crack can follow a path around the tungsten particles, so that it is not necessary to fracture the tungsten particles to weaken the article. Figure 4 is a photomicrograph taken at about 200x magnification of the article in which the tungsten grains are essentially elongated. In elongated tungsten grain articles, the crack cannot transverse the structure of the article without passing through the tungsten particles, and therefore a crack is difficult to propagate. Figure 5 is a schematic diagram showing where crack propagation would occur in such an article. When the article is a kinetic energy penetrator, the penetrator is strengthened as a result of the elongated tungsten grain structure.

The preferred article of this invention is a kinetic energy penetrator. Kinetic energy penetrators must have the strength to resist cracking since high bending stresses which cause cracking are generated when the penetrator hits a target. The target is usually at high obliquity to the path of the penetrator. When the penetrator strikes the target, the penetrator is deflected from its original path and this in effect bends the penetrator and when the length to diameter ratio of the tungsten grains is less than about 2 to 1, the penetrator fractures in a transverse manner. That fracturing reduces its ability to perforate the target. With the elongated grain structure, that is, a length to diameter ratio of at least about 2 to 1, the penetrator is more able to resist fracturing and, therefore, gives better performance.

According to the invention as specified in claim 1 the article is produced by rolling the tungsten heavy alloy body in a tandem rolling mill. One advantage of this method is that the body can be heavily worked without introducing an excessive number of defects to obtain the critical length to diameter ratio.

In operation, the body which has been previously pressed and sintered and which is of the material described previously is rolled in the tandem rolling mill which has a succession of rolling stands, each stand consisting essentially of three rolls positioned at substantially 120_{°} to each other so that the gap between the rolls is a triangle, each stand being rotated about 180_{°} with respect to the adjacent roll stands, so that the resulting rolled article has a hexagonal cross section. The rolling is effected such that the length to diameter ratio of said elongate tungsten grains is at least 2:1. Each stand is calibrated to give a successive reduction in diameter of the body. The amount of reduction in diameter of the body corresponds to the length to diameter ratio of the tungsten grains in the article. Typically a 2.8 to 1 length to diameter ratio corresponds to about a 50% reduction.

A typical procedure for rolling a tungsten heavy metal alloy body according to this invention is given in the examples that ensue.

The three point loading of the body during loading creates a stress system which is not as likely to cause fracture as the more common two point loading rolling mills. High rod rolling speeds such as in excess of about 2000 feet (600 m.) per minute can be attained. Tungsten has a very low specific heat and a high thermal conductivity and, therefore, cools very fast. The rolling speed is fast enough so that the cooling rate is balanced by the heat generated by the deformation process and constant or slightly increasing temperature rolling results.

The rolling is done at a sufficient temperature to produce the article having essentially elongated grains. Temperatures are no greater than about 1000_{°}C and are preferably from about 650_{°}C to about 800_{°}C with about 700_{°}C being especially preferred. If the temperature rises much above about 900°C, microcracking is noticed. If the temperature is lower than the ranges given, there is too much stress on the rolling mill.

The preferred tandem rolling mill is manufactured by Friedrich Kocks and is sold under the name of Kocks Rolling Mill.

One advantage of tandem roll milling is that the article which is generally a long rod can be cut into many small parts. This is opposed to having to press, sinter, and work each individual part.

In order to insure that the article will resist fracturing, the article can be annealed at from about 600_{°}C to about 1400_{°}C depending on the specific properties desired.

To more fully illustrate this invention, the following non-limiting examples are presented.

To roll the tungsten heavy metal alloy body, the following procedure is generally used. First the mill is set up to obtain the amount of rolling required. A typical mill has twelve stand positions. Each stand typically gives a reduction in area of about 18%. the stand calibration is expressed as a plug gauge size. That is, it is the diameter of a body, in particular, a rod that just fits into the gap between the rolls.

### Example 1

Stands having plug sizes of about 0.480, 0.435, 0.394, and 0.357 inch (1 inch = 2.54 cm) are put into the first four stand positions. Bars having a diameter of about 0.526 inch are heated to temperatures of about 300_{°}C, 700_{°}C, and 900_{°}C and fed into the mill. All the bars roll successfully. However, rolling at about 300_{°}C places a high loading on the mill so that this temperature is not desirable. Rolling at about 900_{°}C gives a large number of defects in the rolled rod. Those defects are microcracks which form at the tungsten/nickel alloy (matrix) interface. For these reasons rolling at about 700_{°}C is preferred.

### Example 2

Three additional stands are added to the above stands having plug gauge sizes of about 0.321, 0.281, and 0.300 inch. The latter stand is a finishing stand which has only a10% reduction so that a more uniform hexagon is produced. Bars are heated to about 700_{°}C and fed into the mill and are again rolled successfully. The bars after rolling have a cross sectional area of about 0. 1030 sq. in. giving an overall reduction of about 53%.

### Example 3

Two additional stands having plug gauge sizes of about 0.586 and about 0.530 inch are added to the front (larger diameter) end of the stand line giving a total of nine stands. Bars having a diameter of about 0.700 inch are rolled using a preheat temperature of about 700_{°}C. A total reduction of about 73% is obtained. Therefore, the above three examples show that by increasing the number of stands, the amount of reduction is increased. The work described above is done at a rolling speed of about 300 RPM.

### Example 4

With seven stands in place as in Example 2, tests are run at several rolling speeds, that is, RPM's of the driving motors. At a rolling temperature of about 700°C and an RPM of about 300, the temperature of the bar exiting the mill is about 1000_{°}C which is too high. The RPM is lowered to about 200, 250, and 150. At about 150 RPM, the bar is noticeably colder than at the higher RPM's and the mill becomes overloaded. It is believed that a rolling speed of about 250 RPM is satisfactory.

While there has been shown and described what are at present considered the preferred embodiments of the invention, it will be obvious to those skilled in the art that various changes and modifications may be made therein without departing from the scope of the invention as defined by the appended claims.

## Claims

1. A method of producing an essentially elongate article of tungsten heavy alloy material, said material comprising tungsten, iron and nickel, said method comprising the steps of rolling a pressed and sintered body of said material at a sufficient temperature to produce said article having essentially elongate tungsten grains, characterised in that said rolling is effected in a tandem rolling mill having a succession of roll stands, each stand consisting essentially of three rolls positioned at substantially 120_{°} to each other so that the gap between the rolls is a triangle, each stand being rotated about 180° with respect to the adjacent roll stands, the rolling being effected such that the length to diameter ratio of said elongate tungsten grains is at least 2:1.

2. A method of claim 1 wherein said tungsten heavy alloy material comprises no greater than about 96% by weight tungsten, and nickel and iron in a weight ratio of greater than about 1.5 to 1 Ni to Fe.

3. A method of claim 2 wherein said tungsten heavy alloy material comprises from about 90% to about 96% by weight tungsten, and nickel and iron in a weight ratio of about 7 to 3 of Ni to Fe.

4. A method of claim 1 wherein the temperature is no greater than about 1000°.

5. A method of claim 4 wherein the temperature is from about 650_{°}C to about 800_{°}C.

## Patentansprüche

1. Verfahren zum Herstellen eines im wesentlichen länglichen Gegenstandes aus einem Wolframschwermetallegierungsmaterial, wobei das Material Wolfram, Eisen und Nickel aufweist, wobei das Verfahren die Schritte des Rollens eines gepreßten und gesinterten Körpers dieses Material bei einer Temperatur aufweist, die hinreichend ist, den Gegenstand mit im wesentlichen länglichen Wolframkörnern herzustellen, dadurch gekennzeichnet, daß das Rollen in einer Tandemrollmühle mit einer Folge von Rollenständen durchgeführt wird, wobei jeder Stand aus drei Rollen besteht, die im wesentlichen unter einem Winkel von 120° zueinander angeordnet sind, so daß der Spalt zwischen den Rollen in einem Dreieck ist, wobei jeder Stand um etwa 180° bezüglich dem benachbarten Rollenstand gedreht ist und wobei das Rollen so ausgeführt wird, daß das Verhältnis von Länge zu Durchmesser der länglichen Wolframkömer wenigstens 2:1 beträgt.

2. Verfahren nach Anspruch 1, wobei das Wolframschwermetallegierungsmaterial nicht mehr als etwa 96 Gewichtsprozent Wolfram und Nickel und Eisen in einem Gewichtsverhältnis von nicht mehr als etwa 1,5 zu 1 von Ni zu Fe aufweist.

3. Verfahren nach Anspruch 2, wobei das Wolframschwermetallegierungsmaterial von etwa 90 bis 96 Gewichtsprozent Wolfram und Nickel und Eisen in einem Gewichtsverhältnis von etwa 7 zu 3 von Ni zu Fe aufweist.

4. Verfahren nach Anspruch 1, wobei die Temperatur nicht höher als etwa 1000_{°}C ist.

5. Verfahren nach Anspruch 4, wobei die Temperatur im Bereich von etwa 650_{°}C bis etwa 800_{°}C liegt.

## Revendications

1. Procédé de fabrication d'un produit long en alliage lourd au tungstène, le dit alliage comprenant du tungstène, du fer et du nickel, le dit procédé comprenant l'étape d'un laminage d'un corps pressé et fritté du dit alliage à une température suffisante pour produire le dit produit présentant des particules essentiellement longues de tungstène, caractérisé en ce que le dit laminage est effectué dans un laminoir tandem ayant une succession de trains de laminage, chaque train comportant essentiellement trois rouleaux disposés substantiellement à 120_{°} les uns des autres de manière que l'espace entre les rouleaux forme un triangle, chaque train étant tourné de 180° environ par rapport au train de rouleaux adjacents, le dit laminage étant effectué de telle façon que le rapport de la longueur au diamètre des dites particules longues au tungstène soit au moins égal à 2.

2. Procédé selon la revendication 1 caractérisé en ce que le dit alliage lourd au tungstène comprend moins de 96% environ en poids de tungstène, le nickel et le fer étant présents en poids dans un rapport supérieur à 1,5 à 1 environ.

3. Procédé selon la revendication 2 caractérisé en ce que le dit alliage lourd au tungstène comprend entre 90 et 96% environ en poids de tungstène, le nickel et le fer étant présents en poids dans un rapport de 7 à 3 environ.

4. Procédé selon la revendication 1 caractérisé en ce que la température est inférieure ou égale à 1000° environ.

5. Procédé selon la revendication 4 caractérisé en ce que la température est comprise entre 650 et 800_{°} environ.
